

## UNITED STATES PATENT OFFICE.

GEORGE H. CHARLS, OF CANTON, OHIO, ASSIGNOR TO UNITED ALLOY STEEL CORPORATION, OF CANTON, OHIO, A CORPORATION OF NEW YORK.

## RESISTANT-SURFACE ALLOY OF IRON.

No Drawing.

Application filed April 14, 1924. Serial No. 706,565.

To all whom it may concern:

Be it known that I, GEORGE H. CHARLS, a citizen of the United States, and a resident of Canton, Stark County, State of Ohio, have invented an Improvement in Resist-  
5 ant-Surface Alloys of Iron, of which the following is a specification.

This invention relates to iron alloys. One of the objects thereof is to provide an alloy 10 of iron having a surface adapted to withstand the effect of moisture or other agents without change, and capable of ready manufacture. Another object is to provide an alloy of the above nature which will be 15 strong and tough, and yet readily worked. Other objects will be in part obvious or in part pointed out hereinafter.

The invention accordingly consists in the features and combinations of constituents, 20 all as will be illustratively herein described and the scope of the application of which will be pointed out in the appended claims.

It may first be noted that the term "iron 25 alloy" is used in a broad sense to cover alloys in which carbon may or may not be present, according as it is or is not specified, and thus to include compositions which might with carbon present be more specifically termed a "steel alloy." It is also to 30 be understood that by the expression "resistant surface" is meant a quality of the iron by virtue of which it, throughout its entire mass, is adapted to present a surface which strongly resists the effect of any 35 agencies tending to corrode, discolor, or otherwise alter the same. It may also be noted at this point that in the alloys hereinafter described phosphorus, sulphur and like elements are usually present, as in the 40 case of ordinary commercial iron and steel, but that these elements are to be kept as low as possible.

Considering now an illustrative embodiment of this invention, I have found the 45 following composition to give excellent results: copper from .40% to .60%, molybdenum from .05% to .12%, chromium from 16.0% to 20.0%, and silicon from 1.0% to 2.5%. Carbon, if present, is preferably 50 kept low, and by this is meant, in this connection, that it is preferably substantially below .20%.

Both the copper and molybdenum are also used, for best results, in small quantities,

and it is to be noted that they have a con- 55 joint effect better to a marked degree than that of either used without the other.

I have found as a general rule that excellent results are attained by using the carbon, chromium, silicon and molybdenum in 60 an aggregate amount of from 15.0% to 25.0% of the total.

The ranges above specified are, of course, subject to considerable variation without the loss of much of the beneficial effect in this 65 invention.

There is preferably included in the alloy a small amount of vanadium, say, from .10% to .50%, as a scavenging agent.

The various alloying elements are so 70 added, preferably with the iron in molten form, that they will be thoroughly diffused throughout the mass.

By alloys such as above described the desired character of surface is attained and 75 yet they are readily worked, particularly if the carbon is kept low. Also, no special heat treatment is required.

As a number of variations might be made in the embodiment of my invention above 80 set forth, it is to be understood that all matter herein described is to be interpreted as illustrative and not in a limiting sense.

I claim as my invention:

1. A resistant-surface alloy of iron comprising, in combination with the iron, chromium from 3.0% to 30.0%, silicon from .50% to 6.0%, copper from .10% to 2.0%, and molybdenum from .05% to .35%.

2. A resistant-surface alloy of iron comprising, in combination with the iron, chromium from 3.0% to 30.0%, silicon from .50% to 6.0%, copper from .10% to 2.0%, molybdenum from .05% to .35%, and carbon in an amount not exceeding .20%.

3. A resistant-surface alloy of iron comprising, in combination with the iron, copper from .15% to 2.0%, molybdenum from .05% to .20%, chromium from 3.0% to 25.0%, carbon in an amount not exceeding .20%, and silicon from .50% to 5.00%.

4. A resistant-surface alloy of iron comprising, in combination with the iron, copper from .15% to 2.0%, molybdenum from .05% to .20%, chromium from 16.0% to 25.0%, carbon in an amount not exceeding .20%, and silicon from .50% to 5.00%.

5. A resistant-surface alloy of iron com-

prising, in combination with the iron, copper from .15% to 2.0%, molybdenum from .05% to .20%, chromium from 3.0% to 25.0%, carbon in an amount not exceeding .10%, and silicon from .50% to 5.0%.

6. A resistant-surface alloy of iron comprising, in combination with the iron, copper from .15% to 2.0%, molybdenum from .05% to .20%, chromium from 3.0% to 25.0%, silicon from 1.0% to 4.0%, and carbon in an amount not exceeding .20%.

7. A resistant-surface alloy of iron comprising, in combination with the iron, copper from .20% to .75%, molybdenum from .05% to .20%, chromium from 16.0% to 25.0%, silicon from 1.0% to 4.0%, and carbon in an amount not exceeding .10%.

8. A resistant-surface alloy of iron comprising, in combination with the iron, copper from .40% to .60%, molybdenum from .05% to .12%, chromium from 16.0% to

20.0%, silicon from 1.0% to 2.5%, and carbon from .03% to .07%.

9. A resistant-surface alloy of iron comprising, in combination with the iron, chromium from 3.0% to 30.0%, silicon from .50% to 6.0%, copper from .10% to 2.0%, molybdenum from .05% to .35%, and vanadium in an appreciable amount not exceeding .50%.

10. A resistant-surface alloy of iron comprising, in combination with the iron, copper from .15% to 2.0%, molybdenum from .05% to .35%, chromium from 5.0% to 25.0%, silicon from .50% to 5.0%, carbon in an amount not exceeding .20%, and vanadium in an appreciable amount not exceeding .50%.

In testimony whereof, I have signed my name to this specification this third day 40 of April, 1924.

GEORGE H. CHARLS.